

W. O. SNELLING.  
METHOD OFrecovering METALS.  
APPLICATION FILED SEPT. 18, 1908.  
917,176.

Patented Apr. 6, 1909.



Witnesses:

J. E. Gannett  
Chas. H. Potter

Inventor:

Walter O. Snelling  
By James Townsend & Bickerton,

Atty's:

# UNITED STATES PATENT OFFICE.

WALTER O. SNELLING, OF PITTSBURG, PENNSYLVANIA.

## METHOD OF RECOVERING METALS.

No. 917,176.

Specification of Letters Patent.

Patented April 6, 1909.

Application filed September 18, 1908. Serial No. 453,607.

*To all whom it may concern:*

Be it known that I, WALTER O. SNELLING, a citizen of the United States, residing at Pittsburgh, in the county of Allegheny and 5 State of Pennsylvania, have invented certain new and useful Improvements in Methods of Recovering Metals, of which the following is a specification.

The object of this invention is the provision of a method of recovering metals, in elemental form or as solutions, from their ores, and more particularly from electrically conductive ores. The method is especially adapted for the production of metallic tin 10 from cassiterite and will be described by reference to this particular application. The method is however generally applicable to such ores as are reducible at the cathode in an electrolyte capable of liberating hydrogen.

According to my method the ore, as cassiterite, in suitably subdivided form or in its naturally occurring forms as stream tin, wood tin, etc., is disposed in contact with an electrode in an electrolyte capable of liberating hydrogen. Upon passage of a suitable 20 current reduction of the ore occurs and a part or all of the metal is set free: thereafter the reduced metal is constituted the anode in the same electrolyte, and the metal is dissolved 25 therein and is either deposited upon a suitable cathode, or under suitable conditions is retained in solution.

It will be understood that while in operations of this class the reduction proceeds at 30 first with a high degree of efficiency, this efficiency tends to fall as the operation proceeds, the fall of efficiency being proportionate to the amount of current passing directly to the reduced metal instead of to the unreduced ore. This tendency to reduction of efficiency after the first moments of the operation exists in all cases, but is more pronounced in the treatment of such compounds as are relatively difficult of reduction, easily 40 reducible compounds being more efficient as depolarizers. If the current were merely reversed in the solution after a certain quantity of metal had been reduced at the cathode, and again reversed when this reduced 45 metal had been dissolved and redeposited, no useful purpose would be served, for the metal deposited upon the initial anode would be again dissolved. Therefore in proceeding 50 according to this plan it becomes necessary to remove the deposited metal at the close 55 of each cycle of operations, and such pro-

cedure is costly and troublesome when the reversals are made at short intervals as is required for high efficiency. I prefer therefore to provide in the bath a third or intermediate electrode and to so shift the current connections that one of the three electrodes is at all times cut out of circuit. As hereinafter described, this arrangement permits the cycles to be of very short duration if desired, without however rendering it necessary to remove the deposited metal at correspondingly brief intervals.

A preferred form of apparatus for carrying out my invention is shown in the accompanying drawing wherein the figure is a vertical section of an electrolytic vat, the circuit connection being diagrammatically illustrated.

In said drawing 1 represents a tank or vat consisting of or lined with insulating material adapted for use with the electrolyte selected, and 2, 3, 4, the electrodes therein, the electrode 3 being intermediate the exterior electrodes 2, 4.

5 is a circuit-changing switch which may 80 be of any usual type.

6, 7 represent respectively the positive and negative leads from a direct current circuit of low potential.

Assuming the electrolyte to consist of 85 hydrochloric acid, the several electrodes may consist of graphite: in case sulfuric acid is employed, lead may be used: or a suitable alkaline electrolyte, as caustic soda or sodium stannate, may be employed, in 90 which case the electrodes may be of iron. The plate 2 serves as the anode during the reducing stage, and the perforated plate or screen 3, or the charge thereon in case the ore is conductive, as the initial cathode. 95 When the switch is in the position shown in full lines the current will traverse the bath in such direction as to effect the reduction of the ore, as will be readily understood. When the efficiency of this reduction shows 100 a material decrease as will be the case after the exposed surfaces have been reduced to metal, the switch is moved to the position indicated in dotted lines, whereupon the current will pass from the reduced metal in 105 electrical connection with the plate 3 to the plate or pan 4 as cathode, dissolving the metal and redepositing it. Inasmuch as the reduced metal, as tin, is soluble when connected as anode in the electrolyte chosen, 110 while the material of the plate or screen 3 is insoluble therein, under proper current con-

ditions the current passes almost exclusively from the soluble metal as anode. Inasmuch as the current conditions during the reduction of the ore are not necessarily those which are most appropriate to the solution and deposition of the reduced metal, I prefer to provide a current-controlling device, as for instance a variable resistance indicated at 8, in the electrolyzing circuit. The 10 electrode 4, functioning as cathode during the precipitation, may conveniently be constructed in the form of a shallow removable pan as shown to retain metal deposited in loose or non-adherent form.

15 It will be observed that in the particular arrangement of apparatus described the electrode 2 serves intermittently as anode, and the electrode 4 serves intermittently as cathode, while the intermediate electrode 20 functions alternately as cathode and as anode, the ore undergoing reduction during the first period and the reduced metal being dissolved and redeposited during the second period. Automatic means may be employed 25 for shifting the current connections at intervals suited to the nature of the ore and the character of the current employed, and the process may readily be rendered essentially continuous in character. It will be obvious 30 that the disposition and arrangement of the apparatus may be widely varied without departure from the spirit of my invention.

In case it is desired to produce a solution 35 of a metallic salt, for example stannous chlorid, instead of the metal, this may be accomplished by providing an acid electrolyte, *i. e.* hydrochloric acid, of such concentration as to prevent substantial deposition 40 of the metal during the period that the reduced ore functions as anode.

I claim:

1. The method of recovering metals from 45 their compounds which consists in disposing such compounds in connection with an electrode in a suitable electrolytic bath and reducing portions of the compound to metal, and thereafter connecting said metal as anode in said bath to dissolve the reduced metal.

50 2. The method of recovering metals from their compounds which consists in disposing such compounds in connection with an electrode in a suitable electrolytic bath and reducing portions of the compound to metal, and thereafter connecting said metal as anode in said bath to dissolve the reduced metal and re-deposit the same.

3. The method of recovering metals from 55 electrically conductive compounds which 60 consists in connecting such compound as cathode in a suitable electrolytic bath, reducing portions of the compound to metal, and

thereafter connecting said metal as anode in said bath to dissolve the reduced metal and re-deposit the same.

65 4. The method of recovering tin from its 70 oxid ores which consists in disposing such ore in connection with an electrode in a suitable electrolytic bath, reducing portions of said oxid to metal and thereafter connecting said metal as anode in said bath to dissolve the tin.

75 5. The method of recovering tin from its 80 oxid ores which consists in disposing such ore in connection with an electrode in a suitable electrolytic bath, reducing portions of said oxid to metal and thereafter connecting said metal as anode in said bath to dissolve the tin and re-deposit the same.

70 6. The method of recovering tin from its 85 conductive oxid which consists in connecting the oxid as cathode in a suitable aqueous electrolyte, and electrolytically reducing said oxid.

90 7. The method of recovering metals from 95 their compounds which consists in providing in contact with a suitable electrolyte an electrically intermediate and two electrically exterior electrodes, arranging the compound of the metal in contact with the intermediate 100 electrode, reducing the same by passing an electric current from one of the exterior electrodes as anode, and then shifting the point of supply of current to redissolve said metal and deposit the same on the other of said exterior electrodes.

105 8. The method of recovering tin from its 110 conductive oxid which consists in providing in contact with a suitable electrolyte an electrically intermediate and two electrically exterior electrodes, disposing the oxid in contact with the intermediate electrode, reducing the same by passage of an electric current from one of the exterior electrodes as anode, and then shifting the point of supply of current to redissolve the tin.

95 9. The method of recovering tin from its 115 conductive oxid which consists in providing in contact with a suitable electrolyte an electrically intermediate and two electrically exterior electrodes, disposing the oxid in contact with the intermediate electrode, reducing the same by passage of an electric current from one of the exterior electrodes as anode, and then shifting the point of supply of current to redissolve the tin and deposit the same on the other of said exterior electrodes.

In testimony whereof, I affix my signature in presence of two witnesses.

WALTER O. SNELLING.

Witnesses:

A. L. HYDE,  
HUGO SCHLATTER.